

## UNITED STATES PATENT OFFICE

2,289,300

## PHOTOGRAPHIC SENSITIZER

Gustav Wilmanns, Wolfen, Kreis Bitterfeld, Oskar Riester, Dessau, and Karl Kumetat, Wolfen, Kreis Bitterfeld, Germany, assignors, by mesne assignments, to General Aniline & Film Corporation, New York, N. Y., a corporation of Delaware

No Drawing. Application October 12, 1938, Serial No. 234,604. In Germany October 18, 1937

3 Claims. (Cl. 260—240)

Our present invention relates to photographic sensitizers.

There is a series of sensitizers comprising particularly members of the cyanine-group which serve to sensitize silver halide emulsions for green and green-yellow; that is to say, they are orthochromatic sensitizers. In order to be able to use the brightest light possible in processing the sensitized material in the darkroom, the spectral composition of the light in the darkroom must be shifted as far as possible towards the short wave lengths, i. e. towards bright red or orange. The limit is set on this condition by the initial sensitivity of the emulsion to certain wave lengths. If the sensitizing curve rises from yellow or yellow-green very gradually and flatly, the intensity of the spectral sensitivity at these wave lengths is practically of no importance in working exposures, for it amounts only to a fraction of the intensity of the sensitivity at the sensitizing maximum. This small sensitivity suffices, however, to fog the emulsion when the light of the darkroom falls within that spectral region. Such emulsions, therefore, can only be worked up with correspondingly longer wave lengths, that is to say with light physiologically darker. If, however, a sensitizer is used the sensitizing curve of which falls away as strongly as possible towards the long wave lengths, or a generally more selective sensitizer, the spectral composition of the light in the darkroom may be nearer to the sensitizing zone. Similar advantages of a highly selective sensitizing occur when there is a gap in the green, in which case the processing is conducted in green light.

It is one object of our invention to provide ortho-chromatic emulsions having sensitizing curves which fall away steeply and also have pronounced definite and limited positions of the sensitizing region.

A further object is the provision of trimethinecyanines containing at least one benzimidazole ring.

A still further object is to provide trimethinecyanines with a benzimidazole ring which contains at the nitrogen atoms alkyl, aralkyl or aryl groups.

Other objects of our invention will appear from the description following hereinafter.

The new sensitizers have the following general formula:



in which:

Y=O, S, Se, CH=CH, or

15



R<sub>1</sub>=alkyl,

R<sub>2</sub>=alkyl, aryl, aralkyl or acetoxyalkyl,

X=acid radical, such as Cl, Br, I, SO<sub>4</sub>, ClO<sub>4</sub> or para-toluene sulfonate,

A,B=hydrogen, alkyl or aryl. A and B together may also represent unsubstituted or substituted 25 aryl of the benzene series.

For the production of the unsymmetrical dyestuffs one starts from heterocyclic  $\omega$ -aldehydes, that is to say an aldehyde in which the aldehyde

30 group is a substituent in a methine group attached in 2-position to the nitrogen atom; for example benzthiazole-, benzselenazole-, benzoxazole-, or trimethylindoline-2-methine- $\omega$ -aldehyde may be used. This  $\omega$ -aldehyde is caused

35 to react with 1 mol of 2-methyl-N,N-dialkyl(arylalkyl)-benzimidazolium halide in the presence of a condensing agent, for example pyridine and piperidine.

The dyestuff may contain substituents in the 40 benzene ring. The benzene ring of the benzimidazole may carry a fused-on benzene ring.

The dyestuff is incorporated with the emulsion especially in an emulsion ripened with the use of ammonia emulsion or with the finished layer in 45 any usual manner.

The following examples illustrate the invention:

Example 1.—The unsymmetrical trimethinecyanine produced from 3-ethylbenzthiazole-2-methine- $\omega$ -aldehyde and 1,3-diethyl-2-methyl-6-

ethoxybenzimidazolium iodide and corresponding with the following formula



sensitizes a silver bromide emulsion in the green with a maximum at  $570\text{ m}\mu$  with a very steep falling-away of the sensitivity curve towards the region of long waves.

*Example 2.*—The dyestuff produced from 1.1.3-trimethyl-6-methoxyindoline-2-methine- $\omega$ -aldehyde and 1.3-diethyl-2-methyl-6-ethoxybenzimidazolium iodide and corresponding with the following formula



sensitizes a silver halide emulsion in the green with a maximum at  $545\text{ m}\mu$  and without a gap in the green.

*Example 3.*—The dyestuff obtained by means of 1.1.3-trimethyl-6-methoxyindoline-2-methine- $\omega$ -aldehyde and 1-ethyl-2-methyl-3-phenyl-benzimidazolium iodide and corresponding to the following formula:



sensitizes without a gap in the green and with a maximum at  $560\text{ m}\mu$ .

*Example 4.*—The dyestuff obtained from 1.1.3-trimethylindoline-2-methine- $\omega$ -aldehyde and 1-ethyl-2-methyl-3-phenyl-benzimidazolium iodide has the following formula:



and sensitizes without a gap in the green and with a maximum at  $540\text{ m}\mu$ .

*Example 5.*—The dyestuff produced by means of 3-ethyl-benzselenazole-2-methine- $\omega$ -aldehyde and 1-ethyl-2-methyl-3-phenyl-benzimidazolium ethyl sulfate and corresponding to the following formula:



sensitizes to about  $585\text{ m}\mu$  without a gap and with a maximum at  $557\text{ m}\mu$ .

*Example 6.*—The unsymmetrical dyestuff obtained from 3-ethyl-benzselenazole-2-methine- $\omega$ -aldehyde and 1-ethyl-2-methyl-3-phenyl-6-chloro-benzimidazolium ethyl sulfate and having the following composition:



sensitizes to about  $600\text{ m}\mu$  with a maximum at  $567\text{ m}\mu$ .

*Example 7.*—The unsymmetrical dyestuff obtained from 3-ethyl-benzthiazole-2-methine- $\omega$ -aldehyde and 1-ethyl-2-methyl-3-phenyl-benzimidazolium ethyl sulfate and having the formula:



sensitizes to  $585\text{ m}\mu$  with a maximum at  $555\text{ m}\mu$ .

*Example 8.*—The dyestuff produced from 3-ethyl-benzthiazole-2-methine- $\omega$ -aldehyde and 1-ethyl-2-methyl-3-phenyl-6-chlorobenzimidazolium ethyl sulfate and having the formula:



sensitizes to about  $600\text{ m}\mu$  and with a maximum at  $560$  to  $570$ .

*Example 9.*—The trimethinecyanine produced from 3-ethyl- $\beta,\beta'$ -naphthoxazole-2-methine- $\omega$ -aldehyde and 1-ethyl-2-methyl-3-phenyl-benzimidazolium ethyl sulfate and corresponding with the formula:



sensitizes to  $550\text{ m}\mu$  with a maximum at  $525\text{ m}\mu$ .

*Example 10.*—The trimethinecyanine from 3-ethyl- $\beta,\beta'$ -naphthoxazole-2-methine- $\omega$ -aldehyde and 1-ethyl-2-methyl-3-phenyl-6-chloro-benzimidazolium ethyl sulfate has the formula:



and sensitizes to  $560\text{ m}\mu$  with a maximum at  $538\text{ m}\mu$ .

*Example 11.*—The dyestuff from 1.1.3-trimethylindoline-2-methine- $\omega$ -aldehyde and 1-

ethyl - 2 - methyl-3-(4'-bromophenyl) -6-chloro - benzimidazolium ethyl sulfate has the formula



and sensitizes to 575 m $\mu$  with a maximum at 580 m $\mu$ .

*Example 12.*—The dyestuff obtained by means of 1.1.3-trimethyl-indoline - 2 - methine- $\omega$ -aldehyde and 1-ethyl-2-methyl-3(4'- methoxyphenyl) -benzimidazolium ethyl sulfate has the following formula



and sensitizes to 565 m $\mu$  with a maximum at 540.

*Example 13.*—The dyestuff from 1.1.3-trimethylindoline-2-methine- $\omega$ -aldehyde and 1-ethyl-2-methyl - 3-phenyl - 6 - chloro - benzimidazolium-ethyl sulfate has the formula



and sensitizes to 580 m $\mu$  with a maximum at 550.

*Example 14.*—The dyestuff obtained from 1.1.3 - trimethylindoline - 2 - methine- $\omega$ -aldehyde and 1-ethyl-2-methyl-3-phenyl - 5.6 - dichloro-benzimidazolium ethyl sulfate and corresponding with the following formula



sensitizes to 590 m $\mu$  with a maximum at 560 m $\mu$ .

*Example 15.*—The trimethinecyanine obtained from 1.1.3 - trimethylindoline-2-methine- $\omega$ -aldehyde and 1-ethyl-2.5-dimethyl-3-phenyl-benzimidazolium ethyl sulfate and corresponding with the formula



sensitizes to 565 m $\mu$  with a maximum at 540 m $\mu$ .

*Example 16.*—The trimethinecyanine produced by means of 1.1.3-trimethylindoline-2-methine- $\omega$ -aldehyde and 1-ethyl-2-methyl-3-phenyl-6-

trifluoromethyl-benzimidazolium ethyl sulfate and corresponding with the formula:



10 sensitizes to 580 m $\mu$  with a maximum at 550 m $\mu$ .

*Example 17.*—The trimethinecyanine obtained from 1.1.3-trimethylindoline-2-methine- $\omega$ -aldehyde and 1-ethyl-2-methyl-3-benzyl-6-chloro-benzimidazolium ethyl sulfate and corresponding to the formula



sensitizes to 570 m $\mu$  with a maximum at 542 m $\mu$ .

*Example 18.*—The trimethinecyanine obtained from N-ethyl-thiazoline-2-methine- $\omega$ -aldehyde and 1-ethyl-2-methyl-3-phenyl-6-chloro-benzimidazolium ethyl sulfate and having the formula



sensitizes with a maximum at 510 m $\mu$ .

*Example 19.*—The trimethinecyanine produced from 1.1.3-trimethylindoline-2-methine- $\omega$ -aldehyde and 1-ethyl-2-methyl-3-acetoxy-propyl-6-chloro-benzimidazolium ethyl sulfate and having the following structural formula



sensitizes to 570 m $\mu$  with a maximum at 545 m $\mu$ .

*Example 20.*—The trimethinecyanine produced from N-ethyl-thiazoline-2-methine- $\omega$ -aldehyde, and 1-ethyl-2-methyl-3-acetoxypropyl-6-chloro-benzimidazolium ethyl sulfate has the following structural formula



sensitizes with a maximum at 503 m $\mu$ .

*Example 21.*—The trimethinecyanine produced from 1.2-dimethyl-3-acetoxypropyl-6-chloroben-

zimidazolium methyl sulfate and N-ethyl-benzselenazole-2-methine- $\omega$ -aldehyde having the following formula



and sensitizing to 590 m $\mu$  with a maximum at 15 555 m $\mu$ .

Example 22.—The trimethinecyanine produced from 1-ethyl-2-methyl-3-acetoxypropyl-6-chlorobenzimidazolium-ethyl sulfate and N-ethyl-benzselenazole-2-methine- $\omega$ -aldehyde has the following formula



and sensitizes to 590 m $\mu$  with a maximum at 15 555 m $\mu$ .

Example 23.—The trimethinecyanine produced from 1-ethyl-2-methyl-3-phenyl-6-chlorobenzimidazolium ethyl sulfate and N-ethyl-quinoline-2-methine- $\omega$ -aldehyde has the following formula



and sensitizes to 650 m $\mu$  with a maximum at 15 600 m $\mu$  and a gap at 500 m $\mu$ .

Example 24.—The trimethinecyanine produced from 1-ethyl-2-methyl-3-phenyl-benzimidazolium-ethyl sulfate and N-ethyl-5,6-dimethylbenzselenazole-2-methine- $\omega$ -aldehyde has the following formula



and sensitizes to 590 m $\mu$  with a maximum at 15 563 m $\mu$ .

Example 25.—The trimethinecyanine produced from 1-ethyl-2-methyl-3-phenyl-6-chlorobenzimidazolium-ethyl sulfate and N-ethyl-5,6-di-methylbenzselenazole-2-methine- $\omega$ -aldehyde has the following formula



and sensitizes to 610 m $\mu$  with a maximum at 15 575 m $\mu$ .

Example 26.—The trimethinecyanine produced from 1-ethyl-2-methyl-3-phenyl-benzimidazolium-ethyl sulfate and N-ethyl-5-methoxy-benzselenazole-2-methine- $\omega$ -aldehyde has the following formula



and sensitizes to 600 m $\mu$  with a maximum at 15 565 m $\mu$ .

Example 27.—The trimethinecyanine produced from 1-ethyl-2-methyl-3-phenyl-6-chlorobenzimidazolium-ethyl sulfate and N-ethyl-5-methoxy-benzselenazole-2-methine- $\omega$ -aldehyde has the following formula



and sensitizes to 610 m $\mu$  with a maximum at 15 575 m $\mu$ .

Example 28.—The trimethinecyanine produced from 1-ethyl-2-methyl-3-phenyl-6-chlorobenzimidazolium ethyl sulfate and 1,1,3,6-trimethyl-6-methoxy-indoline-2-methine- $\omega$ -aldehyde has the following formula



and sensitizes to 600 m $\mu$  with a maximum at 15 570 m $\mu$ .

Example 29.—The trimethinecyanine produced from 1-ethyl-2-methyl-3-phenyl-6-chlorobenzimidazolium ethyl sulfate and 1,1,3,6-tetramethyl-indoline-2-methine- $\omega$ -aldehyde has the following formula



and sensitizes to 590 m $\mu$  with a maximum at 15 558 m $\mu$ .

Example 30.—The trimethinecyanine produced from 1,2-dimethyl-3-phenyl-6-chlorobenzimidazolium-methylsulfate and 1,1,3,6-trimethyl-indoline-2-methine- $\omega$ -aldehyde has the following formula



and sensitizes to 580 m $\mu$  with a maximum at 15 550 m $\mu$ .

Example 31.—The trimethinecyanine produced from 1-ethyl-2-methyl-3-(4'-chlorophenyl)ben-

zimidazolium ethyl sulfate and 1.1.3-trimethyl-indoline-2-methine- $\omega$ -aldehyde has the following formula



and sensitizes to 570 m $\mu$  with a maximum at 540 m $\mu$ .

*Example 32.*—The trimethinecyanine produced from 1-ethyl-2-methyl-3-(4'-chlorophenyl)-benzimidazolium-ethyl sulfate and 1.1.3.6-tetramethyl-2-methine- $\omega$ -aldehyde has the following formula



and sensitizes to 575 m $\mu$  with a maximum at 548 m $\mu$ .

*Example 33.*—The trimethine cyanine produced from 1-ethyl-2-methyl-3-(4'-chlorophenyl)-benzimidazolium ethyl sulfate and N-ethyl-thiazoline-2-methine- $\omega$ -aldehyde has the following formula



and sensitizes from 450 to 510 m $\mu$  with a maximum at 493 m $\mu$ .

*Example 34.*—The trimethinecyanine produced from 1-ethyl-2-methyl-3-(4'-chlorophenyl)-benzimidazolium ethyl sulfate and N-ethyl-5.6-dimethyl-benzselenazole-2-methine- $\omega$ -aldehyde has the following formula



and sensitizes to 600 m $\mu$  with a maximum at 565 m $\mu$ .

*Example 35.*—The trimethinecyanine produced from 1-ethyl-2-methyl-3-(4'-methoxyphenyl)-benzimidazolium-ethyl sulfate and N-methyl-5.6-

dimethyl-benzselenazole-2-methine- $\omega$ -aldehyde has the following formula



15 and sensitizes to 595 m $\mu$  with a maximum at 562 m $\mu$ .

*Example 36.*—The trimethinecyanine produced from 1-propyl-2-methyl-3-phenyl-6-chlorobenzimidazoliumiodide and 1.1.3-trimethyl-indoline-2-methine- $\omega$ -aldehyde has the following formula



25 and sensitizes to 580 m $\mu$  with a maximum at 550 m $\mu$ .

*Example 37.*—The trimethinecyanine produced from 1-ethyl-2-methyl-3-phenyl-6-chloro-benzimidazolium-ethyl sulfate and N-propyl-1.1-dimethyl-indoline-2-methine- $\omega$ -aldehyde has the following formula



35 and sensitizes to 580 m $\mu$  with a maximum at 550 m $\mu$ .

*Example 38.*—The trimethinecyanine produced from 1-ethyl-2-methyl-3-phenyl-5-chloro-benzimidazolium ethyl sulfate and 1.1.3-trimethyl-indoline-2-methine- $\omega$ -aldehyde has the following formula



55 and sensitizes to 580 m $\mu$  with a maximum at 550 m $\mu$ .

*Example 39.*—The trimethinecyanine produced from 1-ethyl-2-methyl-3-phenyl-5-chloro-benzimidazolium-ethylsulfate and N-ethyl-thiazoline-2-methine- $\omega$ -aldehyde has the following formula



70 and sensitizes from 450 to 525 m $\mu$  with a maximum at 503 m $\mu$ .

*Example 40.*—The trimethinecyanine produced from 1-ethyl-2-methyl-3-(4'-methoxyphenyl)-benzimidazolium ethyl sulfate and N-ethyl-thiazoline-2-methine- $\omega$ -aldehyde has the following formula



and sensitizes from 450 to 510 m $\mu$  with a maximum at 439 m $\mu$ .

*Example 41.*—The trimethinecyanine produced from 1-ethyl-2-methyl-3-phenyl-5,6-dichlorobenzimidazolium-ethylsulfate and N-ethyl-thiazoline-2-methine- $\omega$ -aldehyde has the following formula



and sensitizes from 450 to 530 m $\mu$  with a maximum at 508 m $\mu$ .

*Example 42.*—The trimethinecyanine produced from 1-ethyl-2-methyl-3-phenyl-benzimidazolium ethyl sulfate and N-ethyl-thiazoline-2-methine- $\omega$ -aldehyde has the following formula



and sensitizes from 450 to 510 m $\mu$  with a maximum at 493 m $\mu$ .

*Example 43.*—The trimethinecyanine produced from 1-ethyl-2-methyl-3-(4'-bromophenyl)-benzimidazolium ethyl sulfate and 1,1,3-trimethylindoline-2-methine- $\omega$ -aldehyde has the following formula



and sensitizes to 560 m $\mu$  with a maximum at 540 m $\mu$ .

*Example 44.*—The trimethinecyanine produced from 1-ethyl-2-methyl-3-(4'-bromophenyl)-benzimidazolium ethyl sulfate and N-ethyl-thiazo-

line-2-methine- $\omega$ -aldehyde has the following formula



and sensitizes from 450 to 510 m $\mu$  with a maximum at 493 m $\mu$ .

*Example 45.*—The trimethinecyanine produced from 1-propyl-2-methyl-3-phenyl-6-chloro-benzimidazolium-iodide and N-ethyl-thiazoline-2-methine- $\omega$ -aldehyde has the following formula



and sensitizes from 450 to 520 m $\mu$  with a maximum at 503 m $\mu$ .

*Example 46.*—The trimethinecyanine produced from 1-ethyl-2,5-dimethyl-3-phenyl-benzimidazoline-ethyl-sulfate and N-ethyl-thiazoline-2-methine- $\omega$ -aldehyde has the following formula



and sensitizes from 450 to 510 m $\mu$  with a maximum at 493 m $\mu$ .

*Example 47.*—The trimethinecyanine produced from 1-propyl-2-methyl-3-phenyl-benzimidazolium-iodide and N-ethyl-thiazoline-2-methine- $\omega$ -aldehyde has the following formula



and sensitizes from 450 to 510 m $\mu$  with a maximum at 493 m $\mu$ .

*Example 48.*—The trimethinecyanine produced from 1-ethyl-2-methyl-3-(4'-chlorophenyl)-6-chloro-benzimidazolium ethyl sulfate and 1,1,3-trimethyl-indoline-2-methine- $\omega$ -aldehyde has the following formula



and sensitizes to 580 m $\mu$  with a maximum at 550 m $\mu$ .

*Example 49.*—The trimethinecyanine produced from 1-ethyl-2-methyl-3-phenyl-6-chlorobenzimidazolium ethyl sulfate and 1.1.3-trimethyl-6-chloro-indoline-2-methine- $\omega$ -aldehyde has the following formula



and sensitizes to 580 m $\mu$  with a maximum at 550 m $\mu$ .

*Example 50.*—The trimethinecyanine produced from 1-ethyl-2-methyl-3-(4'-chlorophenyl)-6-trifluoromethyl-benzimidazolium ethyl sulfate and 1.1.3-trimethyl-indoline-2-methine- $\omega$ -aldehyde has the following formula



and sensitizes to 580 m $\mu$  with a maximum at 550 m $\mu$ .

*Example 51.*—The trimethinecyanine produced from 1-ethyl-2-methyl-3-acetoxypropyl-benzimidazolium ethyl sulfate and 1.1.3-trimethyl-indoline-2-methine- $\omega$ -aldehyde has the following formula



and sensitizes to 550 m $\mu$  with a maximum at 528 m $\mu$ .

*Example 52.*—The trimethinecyanine produced from 1-ethyl-2-methyl-3-acetoxypropyl-benzimidazolium ethyl sulfate and N-ethyl-thiazoline-2-methine- $\omega$ -aldehyde has the following formula



and sensitizes from 450 to 510 m $\mu$  with a maximum at 493 m $\mu$ .

*Example 53.*—The trimethinecyanine produced from 1-ethyl-2-methyl-3-acetoxypropyl-6-chloro-benzimidazolium ethyl sulfate and 1.1.3.6-

tetramethyl-indoline-2-methine- $\omega$ -aldehyde has the following formula



and sensitizes to 575 m $\mu$  with a maximum at 540 m $\mu$ .

*Example 54.*—The trimethinecyanine produced from 1-ethyl-2-methyl-3-acetoxypropyl-6-chloro-benzimidazolium-ethyl sulfate and 1.1.3-tri-20 methyl-6-methoxy-indoline-2-methine- $\omega$ -aldehyde has the following formula



and sensitizes to 585 m $\mu$  with a maximum at 550 m $\mu$ .

*Example 55.*—The trimethinecyanine produced from 1.2-dimethyl-3-acetoxypropyl-6-chloro-benzimidazolium-methylsulfate and N-ethyl-thiazoline-2-methine- $\omega$ -aldehyde has the following formula



and sensitizes from 450 to 520 m $\mu$  with a maximum at 498 m $\mu$ .

*Example 56.*—The trimethinecyanine produced from 1-ethyl-2-methyl-3-acetoxyethyl-6-chloro-benzimidazolium ethyl sulfate and N-ethyl-thiazoline-2-methine- $\omega$ -aldehyde has the following formula



and sensitizes from 450 to 520 m $\mu$  with a maximum at 498 m $\mu$ .

*Example 57.*—The trimethinecyanine produced from 1.2-dimethyl-3-acetoxyethyl-6-chloro-benzimidazolium-methylsulfate and N-ethyl-thiazole-

line-2-methine- $\omega$ -aldehyde has the following formula



and sensitizes from 450 to 520 m $\mu$  with a maximum at 498 m $\mu$ .

Example 58.—The trimethinecyanine produced from 1-ethyl-2-methyl-3-benzyl-benzimidazolium-ethylsulfate and 1.1.3-trimethyl-indoline-2-methine- $\omega$ -aldehyde has the following formula



and sensitizes to 550 m $\mu$  with a maximum at 530 m $\mu$ .

Example 59.—The trimethinecyanine produced from 1-ethyl-2-methyl-3-acetoxyethyl-6-chlorobenzimidazolium ethyl sulfate and N-methyl-thiazoline-2-methine- $\omega$ -aldehyde has the following formula



and sensitizes from 450 to 520 m $\mu$  with a maximum at 498 m $\mu$ .

Example 60.—The trimethinecyanine produced from 1-ethyl-2-methyl-3-isobutyl-6-chlorobenzimidazolium ethyl sulfate and N-ethyl-thiazoline-2-methine- $\omega$ -aldehyde has the following formula



and sensitizes from 450 to 520 m $\mu$  with a maximum at 498 m $\mu$ .

Example 61.—The trimethinecyanine produced from 1.2-dimethyl-3-isobutyl-6-chloro-benzimi-

dazolium-methylsulfate and N-ethyl-thiazoline-2-methine- $\omega$ -aldehyde has the following formula



and sensitizes from 450 to 520 m $\mu$  with a maximum at 498 m $\mu$ .

Example 62.—The trimethinecyanine produced from 1-ethyl-2-methyl-3-acetoxypropyl-4-chloro-benzimidazolium ethyl sulfate and 1.1.3-trimethyl-indoline-2-methine- $\omega$ -aldehyde has the following formula



and sensitizes to 560 m $\mu$  with a maximum of 630 m $\mu$ .

Example 63.—The trimethinecyanine produced from 1.2-dimethyl-3-acetoxypropyl-4-chlorobenzimidazolium-methylsulfate and N-ethyl-thiazoline-2-methine- $\omega$ -aldehyde has the following formula



and sensitizes from 450 to 510 m $\mu$  with a maximum at 493 m $\mu$ .

Example 64.—The trimethinecyanine produced from 1.2-dimethyl-3-acetoxypropyl-6-chlorobenzimidazolium-methyl sulfate and 1.1.3.6-tetramethyl-indoline-2-methine- $\omega$ -aldehyde has the following formula



and sensitizes to 575 m $\mu$  with a maximum at 540 m $\mu$ .

Example 65.—The trimethinecyanine produced from 1.2-dimethyl-3-acetoxypropyl-benzimid-

azolium-methylsulfate and N-ethyl-thiazoline-2-methine- $\omega$ -aldehyde has the following formula



sulfate and N-ethyl-thiazoline-2-methine- $\omega$ -aldehyde has the following formula



10 and sensitizes from 450 to 520 m $\mu$  with a maximum at 490 m $\mu$ .

Example 70.—The trimethinecyanine produced from 1-ethyl-2,3-dimethyl-benzimidazolium-ethyl-sulfate and N-ethyl-thiazoline-2-methine- $\omega$ -aldehyde has the following formula

and sensitizes from 450 to 520 m $\mu$  with a maximum at 493 m $\mu$ .

Example 66.—The trimethinecyanine produced from 1,2-dimethyl-3-benzyl-6-chloro-benzimidazolium-methylsulfate and N-ethyl-thiazoline-2-methine- $\omega$ -aldehyde has the following formula



20 and sensitizes from 450 to 520 m $\mu$  with a maximum at 490 m $\mu$ .

Example 71.—The trimethinecyanine produced from 1,2,3-trimethyl-benzimidazolium-methylsulfate and N-ethyl-benzselenazole-2-methine- $\omega$ -aldehyde has the following formula

and sensitizes from 450 to 525 m $\mu$  with a maximum at 500 m $\mu$ .

Example 67.—The trimethinecyanine produced from 1-ethyl-2-methyl-3-isobutyl-6-trifluoromethyl-benzimidazolium ethyl sulfate and N-ethyl-thiazoline-2-methine- $\omega$ -aldehyde has the following formula



35 and sensitizes to 580 m $\mu$  with a maximum at 545 m $\mu$ .

Example 72.—The trimethinecyanine produced from 1-ethyl-2-methyl-3-(4'-methylmercapto-phenyl)-6-chlor-benzimidazolium-ethyl sulfate and 1,1,3-trimethyl-indoline-2-methine- $\omega$ -aldehyde has the following formula

and sensitizes from 450 to 525 m $\mu$  with a maximum at 500 m $\mu$ .

Example 68.—The trimethinecyanine produced from 1-ethyl-2-methyl-3-isobutyl-6-trifluoromethyl-benzimidazolium ethyl sulfate and 1,1,3-trimethyl-indoline-2-methine- $\omega$ -aldehyde has the following formula



50 and sensitizes to 580 m $\mu$  with a maximum at 545 m $\mu$ .

Example 73.—The trimethinecyanine produced from 1-ethyl-2-methyl-3-dodecyl-6-chlorobenzimidazolium-ethylsulfate and 1,1,3-trimethyl-indoline-2-methine- $\omega$ -aldehyde has the following formula

and sensitizes to 570 m $\mu$  with a maximum at 540 m $\mu$ .

Example 69.—The trimethinecyanine produced from 1,2,3-trimethyl-benzimidazolium-methyl-

75 and sensitizes to 570 m $\mu$  with a maximum at 540 m $\mu$ .

Example 74.—The trimethinecyanine produced from 1,2-dimethyl-3-dodecyl-6-chlorobenzimidazolium-methylsulfate and N-ethyl-benzselen-

zole-2-methine- $\omega$ -aldehyde has the following formula



5

Y is a member selected from the group consisting of O, S, Se, and



D is an o-phenylene radical,

E is a member selected from the group consisting of  $-\text{CH}_2-\text{CH}_2-$ , an o-phenylene radical, and an o-naphthylene radical.

2. A trimethinecyanine corresponding with the following formula:



10

20

and sensitizes to 590 m $\mu$  with a maximum at 560 m $\mu$ .

Example 75.—The trimethinecyanine produced from 1,2-dimethyl-3-dodecyl-6-chlorobenzimidazolium-methylsulfate and N-ethyl-thiazoline-2-methine- $\omega$ -aldehyde has the following formula



in which X is an acid radical.

3. A trimethinecyanine corresponding with the following formula:



in which X is an acid radical.

and sensitizes from 450 to 520 m $\mu$  with a maximum at 500 m $\mu$ . In the above formulae x stands for an alkyl sulfate radical such as ethyl or methyl sulfate.

We claim:

1. A trimethinecyanine corresponding with the following general formula:



30

35

in which  
 R<sub>1</sub> is ethyl,  
 R<sub>2</sub> is acetoxyalkyl,  
 X is an acid radical,

40

GUSTAV WILMANNS.  
 OSKAR RIESTER.  
 KARL KUMETAT.

**Certificate of Correction**

Patent No. 2,289,300.

July 7, 1942.

**GUSTAV WILMANNS ET AL.**

It is hereby certified that errors appear in the printed specification of the above numbered patent requiring correction as follows: Page 1, second column, line 44, after the word "ammonia" strike out "emulsion"; same line, after "finished" insert *emulsion*; page 6, first column, lines 19 and 20, for "maximum at 439  $m\mu$ " read *maximum at 493  $m\mu$* ; page 8, second column, lines 33 and 34, for "of 630  $m\mu$ " read *at 630  $m\mu$* ; and that the said Letters Patent should be read with these corrections therein that the same may conform to the record of the case in the Patent Office.

Signed and sealed this 30th day of March, A. D. 1943.

[SEAL]

**HENRY VAN ARSDALE,**  
*Acting Commissioner of Patents.*